

July 25, 1933.

C. W. BENNETT

1,919,194

METHOD OF MAKING A PRINTING SURFACE

Filed April 7, 1931

*Fig. 1*



*Fig. 2*



*Fig. 3*



*C. W. Bennett*  
Inventor

*by*  
*John J. Graver*  
Attorney

## UNITED STATES PATENT OFFICE

CHARLES W. BENNETT, OF DOUGLASTON, NEW YORK, ASSIGNOR, BY DIRECT AND MESNE ASSIGNMENTS, TO PHOTO-CAST, INC., OF ROCHESTER, NEW YORK, A CORPORATION OF NEW YORK

METHOD OF MAKING A PRINTING SURFACE

Application filed April 7, 1931. Serial No. 528,435.

This invention relates to a process of producing newspaper, magazine, or other printed sheets, and has for its object the provision of a printing surface from which the printed sheet is made, in a manner consuming less time and less expense and in a more efficient manner, than the methods used at present.

With these and other objects in view the invention resides in the novel steps and combinations of steps constituting the process as will appear hereinafter and be explicitly pointed out in the claims.

Referring to the accompanying drawing forming a part of this specification in which like legends designate like parts in all the views,

Fig. 1 is an enlarged sectional view illustrating a plate produced according to this invention;

Fig. 2 is an enlarged sectional view illustrating the formation of a cast by gas evolution from the plate shown in Fig. 1; and

Fig. 3 is an enlarged sectional view illustrating the formation of a cast by mechanical separation of the plate from the body of the casting metal.

This invention constitutes an improvement in the art of producing relief printing surfaces, this application constituting a continuation in part of my application for U. S. Letters Patent filed June 9, 1930 under the Serial No. 460,102 and entitled Method of printing. According to the present invention, the copy makeup is assembled in any convenient manner and the image of said copy then transferred to a supporting medium which preferably is a metallic plate.

The supporting medium further is preferably one so that the image of the copy is produced thereon with the plane of the characters in or substantially in the plane of the metal plate. That is to say, the characters in the image lie in a plane which may be the plane of the metal itself or a plane substantially parallel thereto, the latter being the case if and when the plate is prepared with a coating upon which the image is transferred. This will leave the spaces between the characters on the supporting medium in slightly relief relation which relief will sub-

sequently be increased to a depth necessary for the preparation of the cast containing the printing surface and from which the printed sheet is produced.

The space between the characters just referred to is covered with a material of measurable thickness which, as just stated, may be increased, and said material preferably comprises a heat insulating medium adapted to evolve a gas upon application of heat, for a purpose presently to appear. This gas evolution may result from a chemical change taking place within the substance on the plate, or it may result from a chemical decomposition brought about by heat upon a solid or a liquid applied to the external surface of the plate, in the latter case the heat driving off the occluded or absorbed gas. This material may be for example, powdered glass such as obtained from a Cottrell precipitator in the stack leading from a furnace burning powdered coal, sand, various metallic oxides as for example, iron oxide, various metal salts as for example, copper arsenate, cadmium oxalate, all of which have a relatively high melting point or at least a melting point well above that of the metal of the printing surface.

As an illustration, the copy makeup may be reproduced photographically in a camera upon a bichromated type sensitized surface of the supporting medium, as for example, a copper plate.

The plate is then coated with any suitable varnish such as kettle bodied linseed oil or any other sticky substance and, while sticky, dusted over with any of the materials last mentioned and which are referred to as heat insulating, said dusting penetrating the sticky coating and the excess being brushed off or otherwise removed, after which the plate is developed. That is to say, the material used as the dusting medium will not be confined to the outer surface of the sticky varnish coating but will penetrate said coating even to the gelatin coating on the plate and thereby constituting a path of travel for the water developer to reach the bichromated type sensitized emulsion of the gelatin plate coating. In other words, while the water

naturally would be repelled by the varnish, yet the dusting medium forms a means for conveying the water through the body of the varnish, thus permitting the development of the bichromated plate even after it has been varnished. As a result of the development of the parts of the material, carried by the plate and representing the characters of the copy, will be washed away thus leaving said parts extending through the material to the plane of the plate. In some instances it is desirable to cover or flow over the surface of the developed plate a relatively thin film of a cementitious or flexible material which may be a rubber compound such as from 2 to 6 ounces Pará rubber dissolved in one gallon of solvent such as petroleum naphtha or benzol, the purpose being to assist not only in the adhesion of the metal of the printing surface to the metal of the supporting plate, but also to assist materially in the subsequent formation of relief.

It has been found that a very efficient manner of forming relief is by the creation of gas between the molten metal of the ultimate cast and this supporting plate when the cast is made. Therefore in the selection of the materials above referred to and which occupy the space on the supporting plate between the characters of the image, it is desirable to select those which will give off a gas at the temperatures of the cast. These temperatures will vary dependent on the particular metal of the cast, but with an alloy having a melting point of approximately 70° C., there may be used the Cottrell precipitate above mentioned. The pouring temperature may vary from 100°-400° C. If this gas evolution were not controlled there would be a relatively uniformity of relief in the cast between all characters regardless of the spacing between said characters, as a result of which the casted printing surface would most likely become clogged with the printing ink. Therefore, the use of a film as above indicated, applied over the developed plate, is highly instrumental in confining this gas evolution whereby the gas is held and relief is produced at the same points, which is the point of liberation.

The cast which ultimately contains the printing surface may be made in any suitable manner, the aforementioned plate forming one side of the casting box. In actual practice provision should be made to chill the metal of the plate so that when the molten casting metal, such for example as an alloy consisting of bismuth 50%, lead 25%, tin 12½% and cadmium 12½%, is flowed into the mold, the portion thereof forming the characters of the copy of the printing surface of the cast, will be immediately chilled upon contact with the plane surface of said plate. For example printing relief has been obtained by subjecting the mold

plate to a cooling medium of substantially constant temperature capable of imparting to said plate an initial temperature of 5° C., the temperature of the poured metal being above 190° C. The heat insulating material hereinbefore mentioned will serve to prevent a direct heat transfer from the plate to the molten metal and thus retard the chilling at those parts between the characters of the copy. It thus results that the heat of the casting metal is delayed in reaching the plate and during this delayed time interval the heat of said casting metal is sufficient to affect the relief material on the plate and cause an evolution of gas therefrom. The pressure of this evolved gas pushes the molten casting metal away from the plane of the plate and thus creates an improved relief. A peculiar feature as well as important discovery is, that by the evolution of this gas, the relief in the ultimate cast is made deeper or greater at those parts which correspond to greater separation of characters in the copy. After the cast has cooled sufficiently it is removed from the mold and is then ready for either direct printing or may be used for the preparation of other plates.

It has been found also that high relief is obtained by utilizing a greater difference in temperature of the plate itself while the cast is being made. In other words, more gas is evolved if the plate is externally heated, while the casting metal is in contact therewith, and then subsequently chilled.

While the relief produced according to the above may be sufficient for certain purposes, it may be found desirable to further increase this relief in the following manner. The plate may be prepared as above described or it may be prepared with materials such as pulverized calcium carbonate as well as less finely divided materials previously mentioned, all of which do not give off as much gas as those mentioned and the coating of this material on the plate need not be necessarily of as great thickness as in the preceding case. The film of rubber may also be dispensed with. When the plate is thus prepared it is positioned to form a wall of the casting mold but preferably it is made to assume the upper wall for a purpose as will be readily appreciated from the following. The plate is applied to a frame or other holder which is adapted to maintain the plate in substantially a true plane, a simple frame being a box of which the plate is a cover, said plate covering plural openings in the box connected with a source of vacuum pressure. If an iron or steel plate is used the vacuum pressure would be supplanted with magnets, the idea being to utilize any means for maintaining the plate in a true plane. Further, provision is made in the plate holder for applying the chilling medium to the back side of the plate.

The plate with its holder is then applied to the mold, preferably as the upper wall thereof and the molten casting metal flowed into the mold. Then the plate is chilled. As herein before pointed out, the molten metal in contact with the metal of the plate at those places corresponding to the characters of the copy, will be chilled first, and by proper control of the casting metal and the chilling of the plate, the metal of the cast corresponding to the printing surface is solidified and adheres to the plate. In the preparation of these casts it will, of course, be understood that the relationship of temperatures of the chilling medium and the casting metal will be varied in accordance with the alloy of said metal. In other words for practical purposes it is believed that the temperature of the plate should not be greater than 20° C. and the temperature of the casting metal should be no less than 100° C. As a specific example, a very satisfactory high relief cast was obtained with initial mold plate temperature at -15° C. and casting temperature of 200° C. The coating material on the plate will, through the heat of the casting metal, give off gas as above pointed out but when such materials are used when the gas evolution is small, or when greater relief than hereinbefore pointed out is desired, additional relief is obtained by a separation of the plate from the casting metal before the latter has completely solidified. When the plate is so separated the casting metal will adhere to the plate at the places of the characters so that the cast of the characters is withdrawn from the body of the casting metal, but in this movement the casting metal does not adhere to the spaces on the plate between the characters and therefore is not withdrawn. In practice a draw of as much as one quarter inch has been obtained which gives a remarkable relief.

The separation referred to may comprise a withdrawal of the plate from the still molten casting metal and such withdrawal can be made to give an undercut to the characters in the ultimate cast. In other words, if the plate is withdrawn rapidly relative to the chilling of the plate, undercutting results. With the usual practices of printing, however, this undercutting is not generally desired and therefore the withdrawal of the plate is made less rapidly, relative to the chilling, whereby there results the ultimate formation of characters on the cast with the required slope to the sides. It is to be understood, of course, that the mass of the cast will be sufficiently cooled to be solidified before the plate is broken away from the cast, and this may be accomplished or expedited by a second chilling of the mold, but preferably the mass of the casting metal is not chilled until the proper relief is obtained through the withdrawal of the plate. The

adhesion of the printing surface of the cast to the plate may be varied through the utilization of various films or coatings over the entire surface, as above mentioned.

The principles of the above may likewise be utilized in a reversal of the operation. In other words, after the mold is filled with molten metal, the plate need not be withdrawn but, after the initial chilling and solidification of the printing surface of the cast, a portion of molten metal may be withdrawn from the mold and accomplish the same result of increased relief. From these withdrawals either of the plate, or the metal, it will thus be seen that heat is withdrawn from the molten metal by conduction through the characters themselves and therefore the amount of relief formed is self adjusted. Where the characters are close together heat is withdrawn at a relatively more rapid rate than where the characters are far apart. This means that where the characters are close together the cooling will go forward to the point of bridging across between the characters with solidified metal earlier than in the case where the characters are further apart. In other words, a further withdrawal of molten metal will occur in the case where the characters are further apart than where they are close together, thereby yielding more relief in the former case than in the latter, thus rendering the process a means of obtaining very high relief where this is required and adjusting itself automatically downward where high relief is unnecessary. It is obvious that the plate may assume the position of one of the vertical sides of the mold when the casting metal is run into the mold so that any gas would not collect against the face of the plate, after which and when the mold was filled, the mold could be turned for the plate to assume the upper wall thereof, and then the plate chilled. In cases where the casting metal was withdrawn from the plate it might be necessary to provide a vent in the upper part of the mold so that the metal would leave the plate except at the characters thereon, such a vent of course, being controlled for opening at the proper time namely, after the initial chilling of the character forming portion of the cast. Through such a vent air or gas of atmospheric or superatmospheric pressure may be admitted as the exigencies demanded.

It is obvious that those skilled in the art may vary the details of construction and arrangements of parts constituting the apparatus as well as the steps and combinations of steps constituting the method, all within the spirit of the invention, and therefore it is not desired to be limited to the foregoing except as may be required by the claims.

What is claimed is:—

1. The method of producing a relief printing surface which consists in chilling to solid-

ification selected portions of a mass of molten metal; and raising said portions to obtain the desired relief.

2. The method of producing a relief printing surface which consists in chilling to solidification portions of a mass of molten metal, said portions corresponding to the characters to be printed; and raising said character portions to obtain the desired relief.

3. The method of producing a relief printing surface which consists in chilling to solidification in a mold portions of a mass of molten metal, said portions governed by contact with a preformed mold surface; and raising said portions to obtain the desired relief.

4. The method of producing a relief printing surface which consists in chilling to solidification in a mold portions of a mass of molten metal, said portions governed by contact with a preformed mold surface; and raising said portions by movement of the mold surface to obtain the desired relief.

5. The method of producing a relief printing surface which consists in chilling to solidification in a mold portions of a mass of molten metal, said portions governed by contact with a preformed mold surface; and raising said portions with respect to the center of gravity of the mass of metal to obtain the desired relief, said raising accomplished by the lowering of the said center of gravity.

6. The method of producing a relief printing surface which consists in chilling to solidification through a preformed plate portions of a mass of molten metal; and raising said portions to obtain the desired relief, said raising accomplished by movement of said plate.

7. The method of producing a relief printing surface which consists in bringing a mass of molten metal into contact with a plate having thereon reproduction of the characters to be printed; said reproductions formed by bare portions of the plate and portions covered by a gas producing substance; and causing relative movement between said plate and the mass of molten metal to obtain the desired relief in the casts of the printing characters, said movement brought about by the evolution of gas from said substance.

8. The method of producing a relief printing surface which consists in bringing a mass of molten metal into contact with a plate having thereon reproductions of the characters to be printed; chilling said plate to solidify the portions of the molten mass in contact with said reproductions; and causing relative movement between the chilled plate and the mass of molten metal to obtain the desired relief in the casts of the printing characters.

9. The method of producing a relief printing surface which consists in bringing a mass of

molten metal into contact with a plate having thereon reproductions of the characters to be printed; chilling said plate to solidify the portions of the molten mass in contact with said reproductions; and moving the said plate relative to the mass of molten metal to obtain the desired relief in the casts of the printing characters.

10. The method of producing a relief printing surface which consists in bringing a mass of molten metal into molding contact with a plate having thereon reproductions of the characters to be printed; chilling said plate to solidify the portions of the molten mass in contact with said reproductions; and withdrawing from the mold a part of the mass of molten metal to obtain the desired relief in the casts of the printing characters.

11. The method of producing a relief printing surface which consists in establishing a plate having bare and covered portions; casting a printing metal on said plate; and causing a separation between the covered portions of said plate and the body of said metal by gas evolved from the covered portions while the metal is contacting the bare portions of said plate.

12. The method of producing a relief printing surface which consists in establishing a plate having bare and covered portions; casting a printing metal on said plate; and causing a separation between said plate and the body of said metal by movement of said plate while the metal is contacting the bare portions of said plate.

13. The method of producing a relief printing surface which consists in establishing a plate having bare and covered portions; casting a printing metal on said plate; and causing a separation between the covered portions of said plate and the body of said metal by movement of the body of said metal while the metal is contacting the bare portions of said plate, said movement brought about by pressure of the gas evolved from the substance on the covered portions of said plate.

14. The method of producing a relief printing surface which consists in obtaining an image of the copy makeup on a plate, the characters of the image appearing as bare metal, the spaces between the characters treated with a material capable of evolving gas when heated; and casting the printing metal in contact with said image whereby the heat of the metal will cause an evolution of gas the pressure of which will produce increased relief of the casted characters.

15. The method of producing a printing surface which consists in photographically producing upon a plate an image of the copy makeup; applying to said image a coating capable of evolving gas when heated; removing said coating from the character portions of said image; and casting the printing metal in contact with the treated image.

whereby the heat of the metal will cause an evolution of gas the pressure of which will produce increased relief of the casted characters.

5 16. The method of producing a relief printing surface which consists in establishing a plate having bare and covered portions, the coating on the covered portions capable of evolving gas when heated; and casting 10 therefrom the printing surface in which the relief is greater than the relief of the plate the difference in amount of relief brought

about by movement of the casting metal under pressure of the evolved gas.

17. The method of producing a relief printing surface which consists in establishing a plate having bare and covered portions; 70 the coating on the covered portions capable of evolving gas when heated; and casting a printing metal on said plate, said metal contacting the bare portions of the plate and separated from the coating of the covered 75 portions by the evolved gas.

CHARLES W. BENNETT.

15

80

20

85

25

90

30

95

35

100

40

105

45

110

50

115

55

120

60

125

65

130